

## UNITED STATES PATENT OFFICE

2,534,314

## MODIFICATION OF WOOL TO INCREASE ITS HARSHNESS AND FULLNESS AND TO DECREASE ITS LUSTER

Stuart E. Swanson, Hartford, Conn., assignor to Bigelow-Sanford Carpet Co., Inc., Thompsonville, Conn., a corporation of Massachusetts

No Drawing. Application November 3, 1947,  
Serial No. 783,842

4 Claims. (Cl. 8—95)

1

The present invention relates to the treatment of wool to improve its physical properties and more particularly to a treatment which will enhance the harshness and fullness or plumpness of the wool while at the same time decreasing its lustre.

In the manufacture of pile fabric floor covering by the established operations peculiar to this field, including the carding, spinning, dyeing, etc. of the fiber, it is necessary that the wool be harsh in texture and of a bushy nature so that the fiber possesses a certain fullness. Such bushiness, plumpness, or fullness is also desirable in most cases in the pile tufts of the completed product, which also in many cases should have a low degree of lustre.

B. A.-type wool is so deficient in the foregoing characteristics that it has not been possible to process it into carpets or rugs by the established procedure and with the equipment presently installed in carpet manufacturing plants which operate successfully with the conventional carpet wools of a harsher and plumper character. Because of the soft, slippery nature of the B. A.-type wools, great care and constant attention must be exercised throughout the processing of the wool and the yarn and the weaving thereof. The resulting product is in a sense a hand-made article and commercial production by the established practice is not feasible.

It is an object of the present invention to provide a process for delustering, harshening and plumping B. A.-type wools thereby to extend their use in the manufacture of pile fabric floor coverings.

By the present invention I provide a process for so modifying these B. A.-type wools that the harshness and the plumpness or fullness of the fiber is so increased, as contrasted with the native, untreated fiber, that the treated wool may be manufactured into pile fabric floor covering on a commercial scale by the conventional procedure and apparatus with only normal attention during the processing. It is possible to manufacture on a commercial basis pile fabric floor coverings consisting entirely of B. A.-type wools modified by my process.

In accordance with the invention the wool, either as raw stock, or partly processed, for example in the form of yarn, is modified by wetting it with a solution containing a mixture of aluminum chloride and sodium thiosulfate in approximately equal proportions by weight.

The following is given as an example of my presently preferred process:

2

A batch of raw B. A. wool stock weighing about 900 pounds is immersed in about 4,000 gallons of a cold aqueous solution containing 45 pounds of aluminum chloride and 45 pounds of sodium thiosulfate, based on the weight of the wool. The solution is brought to the boil and maintained at the boiling point for about 20 minutes. Thereafter, the wool is removed from the bath, rinsed in running tap water and dried. The treated wool can be processed into pile fabric floor covering by the conventional procedures employed with the usual carpet wools with no more than normal care and attention.

If the wool is to be colored, it may be dyed with a neutral or direct dye before or after the treatment of this invention; if it is to be dyed with an acid dye the dyeing operation must be completed before the wool is subjected to this modifying treatment, which then may be conducted as indicated in the foregoing example.

When the wool is treated with the aluminum chloride-sodium thiosulfate liquor by the foregoing procedure the treating compounds are completely or substantially completely exhausted from the bath and the amount of the treating compounds taken up by the wool can be controlled by variation of the amount of the treating compound included in the bath.

Although the amounts of modifying agent indicated above have been found to be effective in modifying the wool in accordance with my invention, I have found that the proportion of modifying agent present in the treating liquid is not critical and may be varied over a substantial range depending upon the degree of modification to be imparted to the wool and upon the temperature and the duration of the treatment. Amounts of the modifying compounds ranging from about 1% to 15% of the weight of the wool of each of the two compounds comprising the modifying agent, preferably about 5% of each, have been found advantageous. When the process is carried out at the boil, about 15% of each of the compounds is the maximum amount required to produce the desired results.

The treatment of the present invention is most useful when applied to the B. A.-type wools because, in this case, it serves to convert a wool which can be used only in minor proportions, if at all, for the manufacture of pile fabric floor coverings, into a wool which can be used substantially in the same way as the conventional carpet wools. However, my treatment is also useful with these conventional carpet wools to enhance their qualities of harshness, and of plump-

ness and fullness which render them amenable to processing into pile fabric floor coverings by the established procedures and equipment. The improvement in these properties, however, is not as great in the case of the conventional carpet wools as it is with the B. A.-type wools. The treatment is also useful with mixtures of wools of different types.

Wool treated by my process may be spun into yarn which may then be woven as the pile of pile floor coverings, notwithstanding the fact that the original stock was largely or entirely a B. A.-type wool which inherently is incapable of being processed on the conventional carpet manufacturing apparatus. Such pile has a coarse harsh texture, a bushiness or fullness, and a lack of lustre far different from the texture and lustre of untreated B. A.-type wool and comparable with the texture, bushiness and lustre of the harsher conventional carpet wools.

Raw wool stock modified by my process may be mixed with conventional carpet wools in all proportions to give a wool mixture suitable for use in forming the pile of pile fabric floor coverings.

By the term "B. A.-type wool" as used herein, I mean wool having the characteristics of "B. A. wool" as regards its soft, slippery nature, its lustre and its lack of harshness and fullness as contrasted with the conventional carpet wools. I use the term "B. A. wool" in its ordinary meaning in the trade, i. e., wool from the Lincoln-type sheep as grown in South America. The "B. A.-type" wools available today consist primarily of B. A. wool and wool from the Lincoln sheep as grown in New Zealand.

Although the specific examples of my process given above by way of illustration and not of limitation relate to procedures in which the wool is immersed in a bath of the treating liquid, it is not intended thereby to exclude other ways of applying the liquid to the wool, such as by sprinkling, spraying, etc.

I claim:

1. The process for imparting to B. A.-type wool

the properties of harshness, plumpness and fullness requisite for conversion of the wool by standard procedures into pile fabric floor coverings and for decreasing its lustre which comprises wetting the wool with a solution containing approximately equal amounts of aluminum chloride and sodium thiosulfate.

2. The process as in claim 1 in which the aluminum chloride is present in an amount between about 1% and 15% of the weight of the wool.

3. The process for imparting to B. A.-type wool the properties of harshness, plumpness and fullness requisite for conversion of the wool by standard procedures into pile fabric floor coverings and for decreasing its lustre, which comprises immersing the wool in a boiling aqueous solution containing aluminum chloride and sodium thiosulfate in approximately equal amounts.

4. The process as in claim 3 in which the aluminum chloride is present to an amount between about 1% and 15% of the weight of the wool.

STUART E. SWANSON.

25

#### REFERENCES CITED

The following references are of record in the file of this patent:

#### UNITED STATES PATENTS

| Number    | Name    | Date          |
|-----------|---------|---------------|
| 1,633,213 | King    | June 21, 1927 |
| 1,839,979 | Lorimer | Jan. 5, 1932  |

#### FOREIGN PATENTS

| Number  | Country       | Date           |
|---------|---------------|----------------|
| 132,696 | Austria       | Apr. 10, 1933  |
| 218,877 | Switzerland   | Apr. 16, 1942  |
| 221,422 | Great Britain | Sept. 11, 1924 |

#### 40 OTHER REFERENCES

Dale: "Mordanting Wool with Aluminum Salts." Iowa State College J. Sci., 1942, vol. 17, pps. 49-50. Abstracted in J. Text. Inst., Oct. 1943, 1 page.